

# UNITED STATES PATENT OFFICE.

CARL BOSCH, OF LUDWIGSHAFEN-ON-THE-RHINE, GERMANY, ASSIGNOR TO BADISCHE ANILIN & SODA FABRIK, OF LUDWIGSHAFEN-ON-THE-RHINE, GERMANY, A CORPORATION.

## PROCESS OF WORKING WITH HYDROGEN UNDER PRESSURE.

1,086,130.

Specification of Letters Patent.

Patented Feb. 3, 1914.

No Drawing.

Application filed June 5, 1913. Serial No. 771,898.

To all whom it may concern:

Be it known that I, CARL BOSCH, citizen of the German Empire, residing at Ludwigshafen - on - the - Rhine, Germany, have invented new and useful Improvements in the Process of Working with Hydrogen Under Pressure, of which the following is a specification.

In operations in which hydrogen is employed under pressure in iron tubes or vessels at high temperatures, if the mechanical solidity of the iron is due to the presence of carbon, the tubes or vessels suffer to such an extent that, after a very short time, they are not able to withstand the high pressure employed. I have found that this is due to the action of the hydrogen on the carbon in such a manner that the carbon is converted into gaseous compounds and thus removed from the iron. In the specification of application for patent Serial No. 691,731, I have stated that the disadvantage can be overcome by taking care that the wall which has to sustain the pressure is maintained at a temperature not essentially exceeding 450° C. and in that case any sort of iron which possesses the requisite mechanical solidity can be employed, whether such iron contains much or little carbon or is free from carbon. In continuing my researches in this direction I have now discovered that operations in which hydrogen is employed under pressures exceeding, say, five atmospheres and at high temperatures, can be carried out when the walls of the tubes or vessels which are supporting the pressure possess a temperature essentially above 450° C., provided the said walls be made of iron in which the requisite mechanical solidity of the metal is secured by alloying therewith a metallic solidity giving element such as chromium, vanadium, tungsten, molybdenum, and the like. In these cases it is indifferent whether the iron employed contains carbon or not, since even if the iron originally contained carbon in addition to one of the aforesaid elements, when the hydrogen in the course of time at

the high temperature and pressure employed causes the removal of the carbon from the iron, the remaining alloy of the iron and 50 element as aforesaid still possesses sufficient mechanical solidity to prevent the tube or vessel from giving way under the conditions obtaining.

As instances of alloys which are suitable 55 for use according to my invention, I mention steel containing 18% of tungsten and 3% of chromium, and steel containing 2.9% of chromium and 0.2% of carbon. I prefer to avoid the use of alloys containing 60 too high a percentage of nickel.

The present invention is of great value when preparing ammonia synthetically from nitrogen and hydrogen with the aid of catalytic agents. 65

Now what I claim is:—

1. The process of working with hydrogen at a raised temperature and at a pressure exceeding five atmospheres, which consists in passing the hydrogen under pressure 70 through an iron tube or vessel the walls of which are maintained at a temperature essentially above 450° C. and contain a metallic solidity giving element.

2. The process of working with hydrogen at a raised temperature and at a pressure exceeding five atmospheres, which consists in passing the hydrogen under pressure through an iron tube or vessel the walls of which are maintained at a temperature essentially above 450° C. and contain a metallic solidity giving element, but are practically free from carbon. 80

3. The process of working with hydrogen at a raised temperature and at a pressure exceeding five atmospheres, which consists in passing the hydrogen under pressure through an iron tube or vessel the walls of which are maintained at a temperature essentially above 450° C. and contain chromium. 85

4. The process of working with hydrogen at a raised temperature and at a pressure exceeding five atmospheres, which con-

sists in passing the hydrogen under pressure through an iron tube or vessel the walls of which are maintained at a temperature essentially above 450° C. and contain chromium, but are practically free from carbon.

In testimony whereof I have hereunto set

my hand in the presence of two subscribing witnesses.

CARL BOSCH.

Witnesses:

J. ALEC. LLOYD,

JOSEPH PFEIFFER.